

C. STOLLBERG.  
SCREW CAP FRUIT JAR.  
APPLICATION FILED JUNE 22, 1908.

1,070,748.

Patented Aug. 19, 1913.

Fig. 1



Fig. 2



Fig. 3



Fig. 4



Fig. 5.



Witnesses:

Wm. Geiger  
A. M. Monday

Inventor:  
Charles Stollberg

By Monday, Evans, Adcock & Clarke.  
Attorneys

# UNITED STATES PATENT OFFICE.

CHARLES STOLLEBERG, OF TOLEDO, OHIO, ASSIGNOR TO AMERICAN CAN COMPANY, OF NEW YORK, N. Y., A CORPORATION OF NEW JERSEY.

## SCREW-CAP FRUIT-JAR.

1,070,748.

Specification of Letters Patent. Patented Aug. 19, 1913.

Application filed June 22, 1908. Serial No. 439,686.

*To all whom it may concern:*

Be it known that I, CHARLES STOLLEBERG, a citizen of the United States, residing in Toledo, in the county of Lucas and State of Ohio, have invented a new and useful Improvement in Screw-Cap Kruit-Jars, of which the following is a specification.

My invention relates to improvements in screw caps for fruit or other food preserving jars.

Heretofore screw caps for fruit jars of the kind most commonly and extensively used, have ordinarily been made of sheet zinc, the cylindrical or substantially upright wall being internally screw threaded to engage the external screw threads on the neck of the glass jar, and the flat or disk portion of the cap being lined on the inside with porcelain or other vitreous material to prevent the fruit, vegetables or other food products in the jar from coming in contact with the metal or zinc and thus producing injurious zinc or other salts. As it is, however, the flange or lower edge of the screw cap which engages the shoulder of the jar and compresses the interposed gasket to hermetically seal the jar, there is necessarily always left a certain amount of play or free space, from an eighth to a quarter of an inch, between the upper edge of the jar neck and the lower surface of the porcelain or other vitreous lining of the cap, thus leaving a rim of the zinc exposed to the action of the acid, liquids or gases in the jar; and in fact also the whole upright cylindrical or screw threaded portion of the zinc cap is thus exposed, as such portion does not form a liquid tight engagement with the bottle neck. While the porcelain lining at the flat or disk portion of the screw cap materially diminishes the difficulties arising from the contact of the food contents with the metal of the cap, it is at best but a partial protection or palliative and not a prevention, especially in cases where the fruit jars are inverted, as is customarily done to better insure perfect preservation of the contents; the liquid necessarily coming in contact with the whole screw threaded portion of the cap when the jar is turned upside down. To overcome this difficulty, the screw caps are sometimes made of glass or vitreous material, but they are expensive and liable to breakage, and also defective in operation as

it is very difficult to secure a hermetic closure with certainty and reliability, owing to the unavoidable inequalities in the glass or vitreous cap. And numerous other methods or constructions have been made or attempted to overcome this objection, such, for example, as providing the jar with a double closure, an inner one of glass or vitreous material having a cement or other sealing means, and an outer metal screw cap closure to protect the inner one and insure the hermetic sealing of the jar, but such devices add greatly to the expense of the jar and also to the trouble and labor of sealing the same.

The object of my invention is to provide a screw cap closure for jars which will at once be exceedingly simple and cheap in construction so that its cost will not interfere with extensive use, which can be as readily sealed or closed as the ordinary porcelain lined metal screw cap closure, and which at the same time will absolutely prevent any contamination of or injury to the most delicately flavored fruit or other food contents of the can from the metal of the cap. To practically accomplish this object or result, and herein my invention consists, I employ a screw cap of tin plate, and provide not only its disk portion, but also its upright cylindrical or screw threaded portion with an extremely thin, hard, dry, solid, firmly adherent, impervious, insoluble, innocuous, tasteless and odorless, and at the same time slightly flexible or elastic protective coating, so that the whole interior surface of the sheet metal cap, the screw threaded portion, as well as the disk portion thereof will be fully protected, the thinness, hardness and elasticity of the coating enabling it to extend over the screw threaded portion of the cap without interfering in any way with the action of the screw threads or causing the protective coating itself to be injured by the interengagement of the screw threads on the jar neck and on the cap. This thin, solid, hard, dry, firmly adherent, tasteless, odorless, innocuous, insoluble and impervious protective coating is also preferably extended over the exterior surface of the tin plate screw cap as well as its interior surface, and it is preferably applied while the tin plate sheet from which the screw caps are formed is in the flat. This sanitary protective coating may

be made of any suitable material, having the qualities or characteristics above named. I, however, prefer to use a known coating composed of the following ingredients: 5 per cent. by weight of kauri gum to 80 per cent. by weight of Calcutta linseed oil, to which is added a suitable volatile solvent or reducer, such, for example, as benzin or turpentine in quantity necessary, and to which 10 may also be added a trace of any desired pigment or coloring matter, as for example, asphaltum. This sanitary protective coating which is not herein claimed as a novel composition is preferably applied to the tin 15 plate sheets in the flat in a liquid form and in a thin film extending over the entire surface of the sheets on both sides and then the sheets are preferably baked in a suitable oven for a period of about three hours 20 at a temperature of about three hundred degrees Fahrenheit, thus rendering the protective coating perfectly hard, dry, solid and firmly adherent. After the tin plate sheets are thus prepared, the blanks for the 25 screw caps are cut therefrom and pressed or formed in the required shape in the usual manner.

In the accompanying drawing forming a part of this specification, Figure 1 is a side elevation of a glass fruit jar provided with my improved sheet metal or tin plate protective coated screw cap. Fig. 2 is a vertical section on line 2—2 of Fig. 1. Fig. 3 is a plan view of the cap. Fig. 4 is an enlarged detail section of the cap. Fig. 5 is an enlarged detail section of a portion of the screw cap to indicate the protective coating.

In the drawing, 1 represents a fruit jar, 40 2 its neck having external screw threads 3 and a shoulder 4 forming a seat for the gasket 5, preferably of rubber or other elastic material. The sheet metal screw cap 6 is formed of tin plate having the customary tin coating on both sides of the steel sheet. The screw cap 6 has a flat or disk portion 7 and an upright or cylindrical portion 8 furnished with internal screw threads 9 pressed or formed therein, and an outwardly projecting curved flange or rim 10 at its extreme lower edge to engage the shoulder or gasket seat 4 of the jar, and compress the elastic gasket 5 therebetween, and thus effect a hermetic closure of the jar. The tin 55 plate screw cap is provided on its entire interior surface with an extremely thin, hard, dry, solid, firmly adherent, slightly elastic, innocuous, tasteless, odorless, impervious and insoluble protective coating 11, 60 which extends on the inside of the cap not only over the flat or disk portion 7 thereof, but also over the upright cylindrical or

screw threaded portion 8 thereof, and including the screw threads 9 and flange or rim 10. Owing to the extreme thinness, 65 and hardness of this coating, and its elasticity or freedom from brittleness, I find by experiment, that the interengagement of the screw threads on the cap 6 and jar 1, and the turning of the one set of such threads 70 in respect to the other has no tendency to crack, fray or grind off this protective coating on the screw threads of the metal cap. This protective coating 11 also preferably extends over the entire exterior surface of 75 the cap including the disk portion, the cylindrical portion, the screw threads 9 and flange 10. The outer protective coating adds materially to the life of the sheet metal or tin plate cap and prevents all rusting or 80 tarnishing. Owing to the extreme thinness of the protective coating on the tin plate or sheet metal screw cap and its elasticity, although the same covers every portion of the cap both inside and out, such coating 85 does not interfere with or destroy the natural elasticity of the sheet metal cap or otherwise prevent it from adapting itself to any irregularities of the jar or jar neck to which it is applied. 90

I claim:—

1. A screw cap for fruit jars formed of thin elastic tin plate and having the engaging portion of its screw thread and the interior surface of the cap covered with a hard 95 elastic, tough and protective coating which is innocuous and insoluble overlaid upon the tin plate and impervious to the contents of the jar and capable of resisting the wear on the thread, and adapted to form an elastic 100 closure along the screw thread, substantially as set forth.

2. The combination with a glass fruit jar having its neck furnished with external screw threads, of a thin, elastic sheet metal 105 screw cap of tin plate having its entire interior surface including its screw threads, covered with a thin, hard, elastic, tough and protective coating which is innocuous and insoluble overlaid upon the tin and 110 firmly adherent thereto and impervious to the contents of the jar and capable of resisting the wear on the screw threads, the screw threads of the thin elastic tin plate cap being adapted to conform to the customary irregularities in size and shape of the interengaging external screw threads of the glass 115 jar and cause the cap to form a hermetically tight closure for the jar, substantially as specified.

CHARLES STOLLBERG.

Witnesses:

II. M. MUNDAY,  
PEARL ABRAMS.